# EUROPEAN PATENT SPECIFICATION

(11) **EP 2 657 402 B1**
(45) Date of publication and mention of the grant of the patent: **16.09.2015**
(21) Application number: 13250054.7
(22) Date of filing: 26.04.2013
(51) Int. Cl.: E01C 11/16

(54) **Reinforcing structure and method of manufacture thereof**
Verstärkungsstruktur und Verfahren zu deren Herstellung
Structure de renforcement et son procédé de fabrication

(30) Priority: 28.04.2012 GB 201207576; 14.11.2012 GB 201220439
(43) Date of publication of application: 30.10.2013
(73) Proprietor: Road Solutions Limited, Fall Bank Industrial Estate Dodworth, Barnsley S75 3LS (GB)
(72) Inventor: Inman, Matthew James, Dodworth, Barnsley S75 3LS (GB)
(74) Representative: Atkinson, Ralph

(56) References cited:
- WO-A1-02/12630
- WO-A1-03/087466
- DE-A1-102006 003 085
- JP-A- 2004 314 387
- US-A- 2 115 667

## Description

The present invention relates to a reinforcing structure according to the preamble of claim 1 and a method of manufacture of the same according to the preamble of claim 11.

Reinforcing structures in the form of geosynthetics are currently used in paved structures to provide increased strength and function. Geosynthetics of this type have been developed with the aim of retarding the onset of reflective cracking thereby extending the maintenance cycle of asphalt overlays. They are known to provide sealing, reinforcement, stress relief and adhesive bonding. Conventional geosynthetics are composed of various man-made products and used as reinforcement within asphalt pavements. A problem with such man-made products is that they are not environmentally friendly and often suffer from large carbon footprints. Furthermore, these man-made products often include materials which are harmful to operatives in the field and require additional health and safety measures to be in place during manufacturing procedures and production methods.

An example of a type of reinforcement structure is shown in international patent publication WO 02/12630. This prior art shows a steel mesh reinforcement supported by a crack inducer. The crack inducers create a multitude of fine cracks when concrete is poured over them and additionally provide support for the steel mesh reinforcement. The crack inducers specifically reduces the amount of reinforcement in a slab panel (such as floors, paths and roadways).

International publication WO 03/087466 shows a textile grid of glass, aramid or carbon fibres provided with a coating. The coating includes a plurality of particles, or grains, which increase the surface area of the textile grid. The coating assists in holding the particles in position on the textile grid.

According to an aspect of the present invention, there is provided a reinforcing structure in accordance with claim 1.

A bundle as described herein refers to a plurality of strands of material gathered together. In an embodiment, the strands each comprise a fibre. In a further embodiment, the strands each comprise a filament. In a still further embodiment, the strands each comprise a yarn. In an embodiment, the connection means is in the form of stitching at a crossover point of any one of the first set of bundles with any one of the second set of bundles.

According to a second aspect of the present invention, there is provided a method of manufacturing a reinforcing structure in accordance with claim 11.

The invention will be described by way of example with reference to the accompany drawings, of which:
Figure 1 shows a typical installation scene for applying reinforcing products to a road;
Figures 2A and 2B show a portion of a reinforcing structure embodying an aspect of the present invention;
Figure 3 shows an alternative embodiment to the reinforcing structure shown in Figure 2;
Figure 4 shows a portion of a reinforcing structure suitable for use in the application of Figure 1;
Figures 5A and 5B show a cross sectional view and an exploded isometric view respectively of a reinforcing structure comprising a single carrier layer;
Figures 6A and 6B show a cross sectional view and an exploded isometric view respectively of a reinforcing structure comprising a first carrier layer and a second carrier layer;
Figure 7 shows a cross sectional view of a typical asphaltic paved structure embodying the present invention;
Figure 8 shows a flow chart describing a method of producing a paved surface;
Figures 9A and 9B show an alternative reinforcing structure for use in the paved structures as previously described;
Figure 10 shows a further example of a reinforcing structure for use in the paved structure of Figure 7;
Figure 11 shows a flow chart detailing the manufacture of a reinforcing structure.

### Figure 1

An example embodying the present invention is shown in Figure 1. Figure 1 shows a typical installation scene for applying reinforcing products to a road **101.** It is appreciated that, in an alternative embodiment a pavement, car park or other paved surface can be substituted for the road. In the course of this specification, a paved surface is taken to mean a pavement, car park, road or other firm surface suitable for walking or travelling on. The paved surface may comprise concrete or asphaltic material which may be planed or milled. As shown in the example of Figure 1, a reinforcing structure **102** is laid over a prepared layer **103.** In the embodiment shown, reinforcing structure **102** is in the form of a grid comprising a plurality of bamboo strands and is configured to be positioned at any depth or layer of the road. In the embodiment shown in Figure 1, layer **103** is of the form of a previously laid paved structure. In an alternative embodiment, base layer **103** is a freshly laid layer of asphaltic mixture.

Reinforcing structure **102** is supplied to the site in rolls of the material before being rolled out and laid flat onto the surface of layer **103.** The reinforcing structure is laid flat either by hand or by a suitable mechanical applicator. Once the reinforcing structure **102** has been laid, it can be brushed or rolled and smoothed as required to remove any ripples in the surface. It can also be cut on site as required, particularly around any ironworks present. Once laid, one or more overlaying layers are positioned on top of reinforcing structure **102** to finalise the road structure. The overall road structure and method of laying the road will be discussed in further detail in Figures 7 and 8.

### Figures 2A and 2B

A portion of a reinforcing structure **200** suitable for use in the application of Figure 1 is shown in Figure 2A. Reinforcing structure **200** comprises a first set of bundles **201** which includes bundle **201A,** bundle **201B** and bundle **201C.** Bundle **201A** is arranged substantially parallel to bundle **201B** and bundle **201C.**

Reinforcing structure **200** further comprises a second set of bundles **202,** which includes bundle **202A,** bundle **202B** and bundle **202C.** Second set of bundles **202** is arranged substantially perpendicular to the first set of bundles **201** in a grid **203.** Grid **203** defines a plurality of holes **204,** such as hole **204A.** Hole **204A** has a width indicated by arrow **205** and a length indicated by arrow **206.** In the present embodiment, both the width and the length are substantially similar in size and are greater than 0.004 metres (4mm) in size. Further, the width and the length are preferably less than 0.1 metres (100 millimetres) in size. For example, in an embodiment, the hole size is 0.0125 metres x 0.0125 metres (12.5mm x 12.5mm). In an alternative embodiment the hole size is 0.025 metres x 0.025 metres (25mm x 25mm) and in a still further embodiment the hole size is 0.05 metres x 0.05 metres (50mm x 50mm).

It is appreciated that alternative reinforcing structures that achieve the same objective include holes which are substantially rectangular in shape such that the width is greater than the length or vice versa.

In the embodiment shown, the outer diameter of each one of the first set of bundles 201 is 0.01 metres (10mm), but in alternative embodiments, the bundles have a diameter between 0.002 and 0.03 metres (2 and 30 millimetres). Similarly, the outer diameter of each one of the second set of bundles 202 is 0.01 metres (10 millimetres), and, in a preferred embodiment is between 0.002 and 0.03 metres (2 and 30 millimetres). The specific dimension selected is dependent on the structural requirements of the application in which the reinforcing structure **200** is used for.

Reinforcing structure **200** further comprises a connection means **207** which maintains the first set of bundles **201** and the second set of bundles **202** in grid **203.** In this illustrated example, connection means **207** is in the form of stitching at a crossover point, such as crossover point **208** of bundle **201A** and bundle **202A.** Similarly, bundle **201C** and **202C** are connected together by connection means **209** (in the form of stitching) at crossover point **210.** The stitching comprises a separate piece of material which is tied around the bundles to maintain the bundles in position. In this particular embodiment, the material used for the stitching is derived from bamboo. It is appreciated that similar stitching may or may not be present at any one of the crossover points as shown. It is further appreciated that the stitching may be any other suitable material which will maintain the bundles in position.

Each of the bundles which make up first set of bundles **201** and second set of bundles **202** comprise a plurality of strands of material derived from bamboo. In manufacture, a plurality of strands of material derived from bamboo are obtained and combined to form each bundle. In this illustrated example, therefore, all of the strands of the material comprise a material derived from bamboo.

In some applications of the product, any one of bundles **201** or bundles **202** is provided with a coating which prevents abrasion of the strands when in use. The coating is also configured to protect the strands from excessive heat generated from an overlay of asphalt. An example of the coating is an asphaltic coating and in one such example the coating is polymer modified asphalt. However, in an alternative embodiment, the coating comprises synthetic rubber, for example SBR (styrene butadiene rubber). In a further embodiment, the coating is a polymeric coating such as polyvinyl chloride (PVC), polypropylene (PP) or polytetrafluoroethylene (PTFE). In a still further embodiment, the coating is an epoxy resin, and in a particular example, the epoxy resin is plant-derived epoxy resin. For example, plant-derived epoxy resin can be obtained from plant-derived glycerol which is used to make epichlorohydrin which forms part of the resin. It is appreciated that in other embodiments, the coating is any suitable elastomeric material or naturally occurring polymer suitable for the application required. Figure 2B shows a cross section of the any one of the bundles **201** or **202** where the bundles are provided with a coating **211.** As shown, the bundle comprises a plurality of strands **212** of material derived from bamboo. The coating **211** provides physical and chemical protection to the strands by providing a barrier to the asphaltic layers when positioned in the paving structure.

It is appreciated that, while the portion of reinforcing structure **200** shows a first set of bundles **201** comprising three bundles, in alternative embodiments further bundles are present, with each bundle being positioned substantially parallel to other bundles of the same set. In a particular embodiment only two bundles are present which are arranged in a similar manner.

In the embodiment of Figure 2, the strands of each bundle comprise a fibre or plurality of fibres of bamboo material. It is appreciated however, that in alternative embodiments, the strands of bamboo comprise filaments or a plurality of filaments. Alternatively, the strands of bamboo may comprise a yarn or a plurality of yarns.

While the embodiment herein describes bundles made entirely from material derived from bamboo, in an alternative embodiment, the bundles **201** and **202** further comprise a second material which is combined with the bamboo strands. This second material is any suitable structural material, such as carbon fibre, fibre glass or a polymeric material such as viscose fibres or rayon. Thus, in an embodiment all the strands of the reinforcing structure comprise material derived from bamboo. However, in further embodiments, the strands comprise material derived from bamboo and one or more other materials as described herein.

### Figure 3

An alternative embodiment to the reinforcing structure shown in Figure 2 is shown in Figure 3. In this illustrated example, a portion of reinforcing structure **300** comprises a first set of bundles **301** and a second set of bundles **302.** Each bundle (**301A, 301B, 301C, 301D, 301E** and **301F**) is arranged substantially parallel to each of the other bundles of the set. In this embodiment, each bundle is also paired with another bundle, that is, for example, bundle **301A** is paired with bundle **301B** such that bundle **301A** is positioned a shorter distance from bundle **301B** than to any of the other bundles. Bundle **301A** and bundle **301B** are also arranged substantially parallel to each other. Each pair is also arranged substantially parallel to the other pairs of the reinforcing structure **300.**

Second set of bundles **302** is also arranged such that each bundle (**302A, 302B, 302C** and **302D**) has been paired with another bundle of second set **302.** For example, bundle **302A** is paired with bundle **302B** and bundle **302C** is paired with bundle **302D.** Second set of bundles **302** is arranged substantially perpendicular to the first set of bundles **301.**

First set of bundles **301** and second set of bundles **302** are also arranged in a grid **303.** Grid **303** defines holes, such as hole **304A** and hole **304B.** Hole **304A** has a width **305** and a length **306.** As shown, the width and length are substantially similar in size and define a substantially square hole. In the present embodiment the holes are at least 0.004 metres by 0.004 metres (4mm x 4mm) square, and, preferably, less than 0.1 metres by 0.1 metres (100mm x 100mm) square. In an example, the holes are 0.0125 metres x 0.0125 metres (12.5mm x 12.5mm) in size. In another embodiment the hole length is 0.025 metres (25mm) and the hole width is 0.025 metres (25mm). In a further embodiment, the size of the hole is 0.05 metres x 0.05 metres (50mm x 50mm).

In alternative examples it is appreciated that the holes are substantially rectangular and the widths and lengths are unequal distances. Both the widths and lengths, however, are preferably between 0.004 metres (4 millimetres) and 0.1 metres (100 millimetres) in size.

In order to maintain first set of bundles **301** and second set of bundles **302** in grid **303,** connection means **307** is used. Connection means **307** is in the form of stitching, with stitches used at crossover points, such as crossover point **308,** of any one of the first set of bundles **301** with any one of the second set of bundles **302.** In this illustrated example, crossover point **308** indicates where bundles **302C** and **302D** cross bundles 301E and 301F. As shown, six separate stitches are used to maintain the grid in position. It is appreciated that any other number of stitches can be used as appropriate. The material used for the stitching is a material derived from bamboo.

Each of the bundles shown in Figure 3 comprises a plurality of strands of material derived from bamboo. In the example shown, the strands of material are entirely composed of fibres of bamboo.

In some applications of the product, any one of bundles **301** or bundles **302** is provided with a coating which prevents abrasion of the strands when in use. The coating is also configured to protect the strands from excessive heat generated from an overlay of asphalt. An example of the coating is an asphaltic coating and in one such example the coating is polymer modified asphalt. However, in an alternative embodiment, the coating comprises synthetic rubber, for example SBR (styrene butadiene rubber). In a further embodiment, the coating is a polymeric coating such as polyvinyl chloride (PVC), polypropylene (PP) or polytetrafluoroethylene (PTFE).

In an alternative embodiment to that shown in Figure 3, the strands which make up the bundles comprise both material derived from bamboo and fibre glass. The fibre glass is similar to the type used in conventional paved reinforcing structures. It is understood that different types of fibre glass that are suitable for the purpose can also be used.

In a further embodiment, the strands which make up the bundles comprise both material derived from bamboo and viscose fibres. The viscose fibres can be bamboo derived viscose or an alternative form of viscose. It is further appreciated that the strands may, for example, comprise material derived from bamboo and a combination of fibre glass and viscose fibres. Similarly, the bamboo fibres may be combined with any other suitable structural material, such as carbon or aramid fibres or an alternative polymeric material such as rayon.

It is further appreciated that, while the embodiment described comprises fibres of bamboo, the fibres may be replaced with filaments or yarns of bamboo to achieve the same result.

With reference to the pairing of bundles described previously in this Figure, in an alternative embodiment, more than two bundles are grouped together. In one example, each set of bundles comprises a plurality of grouped bundles wherein each group comprises two or more bundles positioned in relative close proximity to each other. Each group of bundles may also be positioned such that the groups define a hole substantially similar to those previously described.

### Figure 4

Figure 4 shows a portion of a reinforcing structure **400** suitable for use in the application of Figure 1. A section of a grid **401** of reinforcing structure **400** includes a first set of bundles **402** and a second set of bundles **403** arranged to form the grid **401.** The arrangement and composition of the bundles is substantially similar to that previously described in Figure 2.

In the example shown in Figure 4, reinforcing structure **400** further includes a carrier layer **404** which is made of a geotextile material. Carrier layer **404** is a stress absorbing membrane interlayer (SAMI) which is preferably a spun bonded, needle punched or needle bonded material derived from bamboo.

Carrier layer **404** has a mass per unit area of 0.1 kilograms per metre squared (100 grams per metre squared (100 g/m²)) and a tensile strength of between 5000 and 15000 Newtons per metre squared (five and fifteen kilonewtons per metre squared (5-15 kN/m²)). These values are configured to allow the carrier layer to provide a physical barrier from the underlying layer and become saturated with bitumen or asphalt to provide a bond with the overlying layer. For example, the saturation point for 0.1 kilograms (100g) of carrier material is in the region of 0.7 to 1.1 litres per metre square (0.7-1.1 I/m²).

In alternative embodiments, the mass per unit area of the carrier layer is between 0.025 and 0.3 kilograms per metre squared (twenty-five and three hundred grams per metre squared (25-300 g/m²)). In preferred embodiments, the mass per unit area of the carrier layer is 0.05 to 0.1 kilograms per metre squared (fifty to a hundred grams per metre squared (50-100 g/m²)).

In the embodiment shown in Figure 4, the geotextile carrier layer **404** is attached to the grid **401** by stitching to form a single composite material **405.** The stitching is also configured to maintain the grid **401** in position as described previously. The stitching includes a plurality of rows of substantially parallel stitches **406** and a plurality of substantially diagonal stitches **407** positioned between the rows of substantially parallel stitches **406.** The stitches are achieved using suitable knitting machines known in the art for this purpose.

In an alternative embodiment, the grid **401** and the carrier layer **404** are attached by gluing with the two materials combined to form a single material suitable for use in reinforcing a road structure.

The geotextile composite material **405** not only provides both physical and chemical protection for the grid **401** and the bundles **402** and **403** which form the grid, it further provides a backing material which supports the grid when being installed. During installation, the composite material also assists in maintaining the grid in position before asphalt is laid on the top.

### Figures 5A and 5B

Figures 5A and 5B show a cross sectional view and an exploded isometric view respectively of a reinforcing structure **500** akin to that shown in Figure 4. In this embodiment, reinforcing structure **500** comprises a grid **501** and a single carrier layer **502.**

Grid **501** is configured to be substantially similar to any one of the embodiments described in preceding Figures 2, 3 and 4. Carrier layer **502** is substantially similar to that described in Figure 4 and comprises material derived from bamboo. In a preferred embodiment, carrier layer **502** comprises bamboo derived material only. Alternatively, carrier layer **502** further comprises a second material such as glass fibres or viscose fibres.

Grid **501** is attached to carrier layer **502** by stitching, gluing or any other suitable means. In the embodiment shown, carrier layer **502** is attached to a first side **503** of grid **501** with second side **504** remaining exposed to the bitumen or asphaltic layers configured to be laid on top of the reinforcing structure.

### Figures 6A and 6B

In contrast to that shown in Figure 5, Figures 6A and 6B show a cross sectional view and an exploded isometric view respectively of a reinforcing structure **600** comprising a grid **601,** a first carrier layer **602** and a second carrier layer **603.**

Grid **601** is configured to be substantially similar to any one of the embodiments described in preceding Figures 2, 3 and 4. Both first carrier layer **602** and second carrier layer **603** are substantially similar to the carrier layer described in Figure 4 and comprise material derived from bamboo. In a preferred embodiment, each carrier layer comprises bamboo derived material only. In a further embodiment, each carrier layer comprises a second material, for example, glass fibres or viscose fibres. It is appreciated that, dependent on site requirements, each carrier layer can be substantially different to the other in composition, and may comprise a combination of the above.

Referring back to Figure 6, first carrier layer **602** is attached to a first side **604** of grid **601,** while second carrier layer **603** is attached to a second side **605** of grid **601.** Second carrier layer **603** is also positioned in a substantially parallel plane to first carrier layer **602.**

Grid **601** is attached to carrier layer **602** by stitching, gluing or any other suitable means. Grid **601** is also attached to carrier layer **603** by any suitable method including, but not limited to, stitching or gluing.

In the embodiment of Figure 6, a coating is not required on the bundles of grid **601** as the carrier layers **602** and **603** provide the required physical and chemical protection from the asphaltic layers which sandwich reinforcing structure **600** when in use in a paving structure. Carrier layers **602** and **603** are configured to protect grid **601** from abrasion and heat during the laying of hot bitumen. In some applications where stresses are particularly high, however, a suitable coating is used to provide additional protection.

In an embodiment, second carrier layer **603** has a thickness greater than first carrier layer **602.** When positioned in the road or paved structure, the thicker carrier layer is configured to be positioned closest to the surface allowing the upper thicker carrier layer to provide heat insulation. In a preferred embodiment, the upper thicker carrier layer has a mass per unit area of between 0.1 and 0.3 kilograms per metre squared (one hundred and three hundred grams per metre squared (100-300 g/m²)). In contrast, the lower thinner carrier layer has a mass per unit area of between 0.05 and 0.1 kilograms per metre squared (fifty and a hundred grams per metre squared (50-100 g/m²)).

### Figure 7

A cross sectional view of a typical asphaltic paved structure or road section embodying the present invention is shown in Figure 7. Paved structure **701** comprises a plurality of layers including an underlying section **702,** a reinforcing structure **703** and an overlaying section **704.**

Reinforcing structure **703** is positioned between underlying section **702** and overlaying section **704.** Preferably, the reinforcing structure **703** is positioned as far down in the paved structure as possible to provide maximum support to over laying section **704.** Reinforcing structure **703** comprises a textile layer comprising a plurality of bamboo strands. The reinforcing structure **703** is substantially similar to any one of the reinforcing structures previously described and is configured to prevent movement and cracking from the underlying layers from dissipating to the overlying layers when placed in position.

In an embodiment, underlying section **702** comprises a plurality of layers of varying compositions. In the illustrated example, the underlying section comprises a base layer **705** and two sub base layers **706** and **707.** Base layer **705** comprises large aggregate material and contacts a first side **708** of reinforcing structure **702.** First sub base layer **706** comprises a small stone layer, for example a Type 1 sub base. Second sub base layer **707** comprises a large stone sub base layer, for example a Type 2 sub base. In an alternative embodiment, the second sub base layer **707** is omitted.

Overlaying section **704** also comprises a plurality of layers of varying compositions. As shown, overlaying section **704** comprises a lower layer (or binder course) **709** and a surface course **710.** Lower layer **709** is an asphaltic layer and is configured to be in contact with a second side **711** of reinforcing structure **703.** It is anticipated that surface course **710** is a further asphaltic layer which is configured to wear through use. Surface course **710** will be replaced over periods of time due to expected wear and tear. In particular, without reinforcing structure **703** in place, surface course **710** is highly susceptible to cracking.

The paved structure further comprises a bond coat **712** which is positioned between base layer **705** and reinforcing structure **703.** The bond coat comprises pure bitumen or bitumen emulsion or a polymer modified bitumen solution. It is appreciated that an alternative polymer modified solution could be used.

Typically, overlaying section **704** is between 0.085 and 0.150 metres (eighty-five and one hundred and fifty millimetres (85-150 mm)) thick, which corresponds to a thickness of reinforcing structure **703** of 0.002 to 0.040 metres (two to forty millimetres (2-40 mm)).

It is appreciated that the number of layers present in underlying section **702** varies depending on the application required depending on the load bearing capacity requirements (such as the Californian Bearing Ratio (CBR)) of the paved structure. Similarly, overlaying section **704** may comprise any number of suitable layers dependent on the application requirements. In a particular embodiment, underlying section **702** comprises a single layer of suitable material.

Similarly, overlaying section **704** may comprise a single layer of asphaltic material. In an example embodiment, surface course **710** is the only layer of overlaying section **704** and is configured to be in contact with second side **711** of reinforcing structure **703.**

### Figure 8

Figure 8 shows a flow chart describing a method of producing a paved surface.

At step **801** the base layer of the paved surface is prepared. In an example where the base layer is an existing asphaltic or concrete pavement, the surface can be levelled to provide a clean and smooth surface most suitable for laying the reinforcing layer. In an alternative example the base layer has been freshly laid and this step forms part of the standard procedure for laying the base layer.

At this stage, any cracks or other joints are sealed with suitable fillers as necessary and further repairs can be made to ensure a uniform level surface. A further regulating layer may be added if the surface is particularly damaged. The surface is then cleaned as required before moving onto the next step.

At step **802** a uniform layer of a bond coat comprising bitumen is applied or sprayed to leave a residual coating 0.7 metres per square metre (seven hundred millilitres per metre square (700 ml/m²)). In an embodiment, a hot bitumen road emulsion of the type K1-70 (which includes around 70% bitumen and 30% water) is sprayed at a rate of around 1 litre per metre squared (1 l/m²). This rate is increased for surfaces with greater porosity. The bitumen is also configured to saturate the reinforcing layer to enable the reinforcing layer to become an integral piece of the paving structure.

The bond coat may alternatively comprise pure bitumen or bitumen emulsion or a polymer modified solution. In an embodiment, a polymer modified bitumen solution is used.

Spraying of the bond coat is achieved by means of a calibrated spray tanker which enables a uniform spread of the bond coat. Alternatively, the spraying can be achieved by use of hand-held tools, such as a hand lance sprayer.

At step **803,** the reinforcing structure is installed over the top of the bond coat layer. The reinforcing structure comprises a textile layer comprising a plurality of bamboo strands. It is appreciated that any one of the reinforcing structures discussed previously may be used for this purpose. The reinforcing structure is positioned by rolling it out and laid flat onto the prepared surface. The surface is brushed under sufficient tension to ensure the reinforcing structure is laid flat onto the base layer. In an embodiment, the hot bitumen road emulsion is allowed to cure prior to laying any further layers.

In an embodiment where the reinforcing structure comprises two carrier layers, the upper carrier layer may not be fully saturated by the bond coat, particularly where the upper carrier layer is thicker than the lower carrier layer. In this case, the reinforcing structure can be oversprayed with emulsion until saturation occurs and prior to step **804** being conducted.

At step **804,** one or more layers are applied over the reinforcing structure. In an embodiment, a binding course is laid first over the reinforcing structure with a surface layer laid above the binding course. The surface course is compacted asphalt overlay and should have a minimum thickness of 0.040 metres (40mm). In a particular embodiment, the thickness of the overlay is 0.050 metres (50mm).

### Figures 9A and 9B

An alternative reinforcing structure **900** which could be used in the paved structures as previously described and in accordance with the application of Figure 1 is shown in Figure 9. The reinforcing structure **900** comprises a set of reinforcing elements **901** with each reinforcing element arranged in a substantially parallel position relative to each of the other reinforcing elements of the set as shown. In this illustrated example, reinforcing element **901A** is positioned substantially parallel to reinforcing element **901B** and reinforcing element **901C.**

Reinforcing structure **900** further includes a second set of reinforcing elements **902** which are arranged at an angle to set of reinforcing elements **901.** In this illustrated example, the angle is approximately 90°. In other embodiments, however, the angle is any suitable angle for the application in question.

The set of reinforcing elements **901** and the set of reinforcing elements **902** are connected to each other by connection means **903.** In the embodiment of Figure 9, the connection means comprises stitching which holds each of the reinforcing elements together at crossover points, such as crossover point **904.** Alternative connection means are used in other examples, such as those described in Figure 10.

As shown, the reinforcing elements **901** and **902** are spaced such that holes, such as hole **904,** are defined between them.

In the embodiment of Figure 9A, each reinforcing element **901** and **902** is formed of a composite material comprising a plurality of bamboo fibres and a binding matrix. Figure 9B shows a cross sectional view of any one of the reinforcing elements **901** or **902** of the composite material described in reference to Figure 9A. The cross section shows a plurality of bamboo fibres **905** which have been substantially aligned in the process of manufacture (as described further in Figure 11). The bamboo fibres **905** are surrounded by the binding matrix **906** with each of the bamboo fibres being bound to any one or more of the other bamboo fibres by means of the binding matrix.

The binding matrix is any suitable material which can be used in combination with the plurality of bamboo fibres to form a composite material. For example, in an embodiment, the binding matrix is an asphaltic coating and comprises polymer modified asphalt or a bitumen emulsion. In an example embodiment, the binding matrix is produced from a naturally occurring source, and comprises natural resins or material derived from bamboo. In an embodiment, the binding matrix is bamboo sap. In a further embodiment, the binding matrix comprises rubberwood sap or a natural rubber component. In another embodiment, the binding matrix comprises a synthetic rubber, for example, SBR (styrene butadiene rubber). In a further embodiment, the binding matrix comprises a polymeric material such as polyvinyl chloride (PVC), polypropylene (PP) or polytetrafluoroethylene (PTFE). In a still further embodiment, the binding matrix is an epoxy resin, and in a particular example, the epoxy resin is plant-derived epoxy resin. For example, plant-derived epoxy resin can be obtained from plant-derived glycerol which is used to make epichlorohydrin forming part of the resin.

As a part of the composite material, the binding matrix not only works to bind the reinforcing bamboo fibres together, but also works as a coating to provide physical and chemical protection to the bamboo fibres. The binding matrix therefore advantageously works to prevent abrasion of the bamboo fibres and avoids damage to the reinforcing structure from the heat generated from the overlay of asphalt (as described in the paved structure of Figure 7).

In an embodiment, the composite material further comprises fibres of a second material in addition to the bamboo fibres such that the composite material may also include fibres of viscose, glass fibres, carbon fibres or other suitable fibres as previously described.

In a particular embodiment, the composite material is a preimpregnated (pre-preg) material. Thus, the fibres are aligned and impregnated with the binding matrix and partially cured to produce a pre-preg material suitable for the reinforcing structure. This process is explained in further detail in Figure 11.

### Figure 10

A further example of a reinforcing structure suitable for use in the paved structure of Figure 7 and in accordance with the application shown in Figure 1 is shown in Figure 10. Reinforcing structure **1000** comprises a first set of reinforcing elements **1001** which are arranged substantially parallel to the other reinforcing elements of the set. In this illustrated example, reinforcing element **1001A** is positioned substantially parallel to reinforcing element **1001B** and reinforcing element **1001C.**

Reinforcing structure **1000** further comprises a second set of reinforcing elements **1002** which are arranged at an angle to the reinforcing elements of the first set **1001.** In this illustrated embodiment, the angle is approximately 90°. However, it is appreciated that other suitable angles may be used depending on the requirements of the application.

In an embodiment, each reinforcing element (**1001** and **1002**) is formed of a composite material comprising a plurality of bamboo fibres and a binding matrix. The reinforcing elements are connected by a connection means, which, in an embodiment, may be similar to the example shown in previous Figure 9 and include stitching. However, in the embodiment shown in Figure 10, the connection means is configured to be part of the binding matrix itself. In this embodiment, the binding matrix is configured to be tacky in texture, such that each reinforcing element can be positioned in place and fixed to another reinforcing element by forcing the reinforcing elements together. In a further embodiment, a suitable adhesive is used to maintain the reinforcing elements in position with each of the reinforcing elements being glued together.

In the embodiment shown, reinforcing elements **1001** and **1002** are spaced such that holes, such as hole **1003,** are defined between them. In a further embodiment, and to increase strength of the reinforcing structure as required, the reinforcing elements **1001** and **1002** are layered on top of other reinforcing elements and stacked to increase the thickness of the reinforcing structure as a whole.

The binding matrix of the embodiment in Figure 10 is any suitable material which can be used in combination with the plurality of bamboo fibres to form a composite material. For example, in an embodiment, the binding matrix is an asphaltic coating and comprises polymer modified asphalt or a bitumen emulsion. In an example embodiment, the binding matrix is produced from a naturally occurring source, and comprises natural resins or material derived from bamboo. In an embodiment, the binding matrix is bamboo sap. In a further embodiment, the binding matrix comprises rubberwood sap or a natural rubber component. In another embodiment, the binding matrix comprises a synthetic rubber, for example, SBR (styrene butadiene rubber). In a further embodiment, the binding matrix comprises a polymeric material such as polyvinyl chloride (PVC), polypropylene (PP) or polytetrafluoroethylene (PTFE).

As a part of the composite material, the binding matrix not only works to bind the reinforcing bamboo fibres together, but also works as a coating to provide physical and chemical protection to the bamboo fibres. The binding matrix therefore advantageously works to prevent abrasion of the bamboo fibres and avoids damage to the reinforcing structure from the heat generated from the overlay of asphalt (as described in the paved structure of Figure 7).

In an embodiment, the composite material further comprises fibres of a second material in addition to the bamboo fibres such that the composite material may also include fibres of viscose, glass fibres, carbon fibres or other suitable fibres as previously described.

In a particular embodiment, the composite material is a preimpregnated (pre-preg) material. Thus, the fibres (that is, bamboo fibres or fibres composed of both bamboo fibres and at least one further material) are aligned and impregnated with the binding matrix and partially cured to produce a pre-preg material suitable for the reinforcing structure. This process is explained in further detail in Figure 11.

In a further embodiment, the reinforcing structures shown in both Figures 9 and 10 further comprise carrier layers in a similar manner to the embodiments shown in Figures 5 and 6. In a preferred embodiment, each carrier layer is made of a geotextile material and is a stress absorbing membrane interlayer (SAMI) which is preferably a spun bonded, needle punched or needle bonded material derived from bamboo.

In an example embodiment, the reinforcing structure further comprises a single carrier layer which is attached to a first side of at least one of the reinforcing elements. In a further embodiment, the reinforcing structure comprises a further carrier layer, which is attached to a second side of a least one of the reinforcing elements. In this example, the further carrier layer is positioned in a substantially parallel plane to the first carrier layer.

In a particular embodiment, one of the carrier layers has a greater thickness than the other carrier layer such that the thicker layer can be utilised to enable increased protection for the reinforcing elements from the hot bitumen which overlays the reinforcing structure when laid as part of a paved structure.

### Figure 11

Figure 11 shows a flow chart detailing the manufacture of a reinforcing structure comprising a composite grid in accordance with the embodiments described in Figures 9 and 10.

At step **1101** long length bamboo fibres are obtained from natural bamboo by means of mechanical extraction. In a preferred embodiment, the mechanical extraction is purely mechanical and does not include the addition of chemicals or the use of high temperatures so as to prevent damage or weakening of the bamboo fibres. Bamboo fibres of up to 0.35 metres (thirty five centimetres (35 cm)) in length are obtained from the length between the nodes of the natural bamboo by this method.

In an alternative embodiment, the bamboo fibres are extracted from natural bamboo by steam explosion utilising high pressures and temperatures as known in the art. Further embodiments include chemical extraction of the bamboo fibres from natural bamboo by utilising high concentrations of sodium hydroxide (NaOH).

Once the bamboo fibres have been extracted from the culm of the natural bamboo, the fibres are cleaned and aligned at step **1102.** For manufacture of unidirectional composites, the bamboo fibres are combed and arranged such that the fibres are aligned substantially parallel to each other.

At step **1103,** a suitable binding matrix is added. The binding matrix is any suitable material which binds the fibres together and provides a degree of protection from the hot asphaltic mixture of the paved structure. In a preferred embodiment, the binding matrix is an asphaltic coating and comprises polymer modified asphalt or a bitumen emulsion. Alternatively, in an embodiment, the binding matrix is produced from a naturally occurring source, and comprises natural resins or material derived from bamboo. In one embodiment, the binding matrix is bamboo sap. In a further embodiment, the binding matrix comprises rubberwood sap or includes a natural rubber component.

In a further embodiment, the binding matrix comprises a synthetic rubber, for example, SBR (styrene-butadiene rubber). In a still further embodiment, the binding matrix comprises a polymeric material such as polyvinyl chloride (PVC), polypropylene (PP), maleic anhydride grafted polypropylene (MAPP) or polytetrafluoroethylene (PTFE). Alternatively, in an embodiment the binding matrix comprises epoxy resin. In a particular example, the epoxy resin is plant-derived epoxy resin. For example, plant-derived epoxy resin can be obtained from plant-derived glycerol which is used to make epichlorohydrin forming part of the resin.

In an embodiment, layers of bamboo fibres are positioned between layers of film of the binding matrix material before at least partially curing and/or melting. The bamboo fibres and binding matrix in combination are then compression moulded at step **1104** such that the binding matrix is partially cured to form pre-preg composite reinforcing elements. In a preferred embodiment, the bamboo fibres and binding matrix are heated while compression moulded to enable the fibres and matrix to form suitable bonds. It is appreciated that the film of binding matrix can be any of the aforementioned materials described previously and suitable for the particular application.

At step **1105** the pre-preg composite reinforcing elements are aligned as required into a grid or similar form, such as those illustrated in Figures 9 and 10, such that a composite reinforcing structure is obtained. The reinforcing elements may be split into a first set and a second set. The first set of reinforcing elements are then arranged such that each reinforcing element is positioned substantially parallel to the other reinforcing elements in the set. The second set of reinforcing elements are then arranged at an appropriate angle to the first set of reinforcing elements before the two sets are connected together with appropriate connection means. The connection means may take the form of stitching, gluing or other adhesive. In an embodiment, the connection means is that of the binding matrix itself which is used to maintain the reinforcing elements in position.

Once arranged, the reinforcing composite can be used as part of a paved structure such as those described herein.

## Claims

1. A reinforcing structure (200, 300, 400, 500, 600, 703, 900, 1000) comprising:
a first set of bundles (201, 301, 402, 901, 1001), each said bundle arranged substantially parallel to other bundles of said first set;
a second set of bundles (202, 302, 403, 902, 1002) arranged substantially perpendicular to said first set of bundles;
said first set of bundles and said second set of bundles are arranged in a grid (203, 303, 401, 501, 601) defining holes (204, 304, 1003) having widths (205, 305) and lengths (206, 306) greater than 0.004 metres; and
said reinforcing structure further comprising a connection means (207, 307, 407, 903) which maintains said first set of bundles and said second set of bundles in said grid; **characterised in that**
each said bundle comprises a plurality of strands (212, 905) of material derived from bamboo and each said bundle is provided with a coating (211, 906) to provide physical and chemical protection to said strands.

2. A reinforcing structure in accordance with claim 1, wherein said reinforcing structure is formed in a roll of material.

3. A reinforcing structure in accordance with claim 1, wherein said bundles comprise said strands of material derived from bamboo and further comprise strands formed of a second material.

4. A reinforcing structure in accordance with claim 3, wherein said second material is selected from at least one member of the group consisting of: fibre glass, viscose fibres and carbon fibre.

5. A reinforcing structure in accordance with claim 1, further comprising a first carrier layer (404, 502) attached to a first side (503) of said grid.

6. A reinforcing structure in accordance with claim 1, wherein said coating (211) is selected from at least one member of the group consisting of: a polymeric material, an elastomeric material, naturally occurring polymer, polymer modified asphalt, synthetic rubber, naturally occurring bamboo sap, naturally occurring bamboo resin, a natural rubber component, epoxy resin and plant-derived epoxy resin.

7. A reinforcing structure in accordance with claim 1, wherein said strands comprise a first plurality of bamboo fibres (905) and said coating comprises a binding matrix (906).

8. A reinforcing structure in accordance with claim 7, wherein said first plurality of bamboo fibres comprises a second plurality of bamboo fibres and in which each of said second plurality of said bamboo fibres is bound to another one of said second plurality of bamboo fibres by said binding matrix.

9. A reinforcing structure in accordance with claim 7, wherein said connection means comprises said binding matrix (906).

10. An asphaltic paved surface (701) comprising a reinforcing structure (200, 300, 400, 500, 600, 703, 900, 1000) in accordance with any previous claim.

11. A method of manufacturing a reinforcing structure (200, 300, 400, 500, 600, 703, 900, 1000), comprising the sequential steps of:
obtaining a plurality of strands (212, 905) of material derived from bamboo;
combining a plurality of strands to form a first set of bundles (201, 301, 402, 901, 1001) and a second set of bundles (202, 302, 403, 902, 1002);
arranging said first set of bundles such that each said bundle is substantially parallel to a corresponding bundle;
arranging said second set of bundles substantially perpendicular to said first set of bundles;
arranging said first set of bundles and said second set of bundles in a grid (203, 303, 401, 501, 601) defining holes (204, 304, 1003) having widths (205, 305) and lengths (206, 306) greater than 0.004 metres;
connecting said first set of bundles and said second set of bundles to maintain said grid; and
providing said bundles with a coating (211, 906) to provide physical and chemical protection to said strands.

12. A method of manufacturing a reinforcing structure in accordance with claim 11, wherein said plurality of strands comprises a plurality of bamboo fibres and said step of combining said plurality of strands comprises:
refining said plurality of bamboo fibres such that said plurality of bamboo fibres are substantially aligned.

13. A method of manufacturing a reinforcing structure in accordance with claim 12, wherein said step of providing said bundles with a coating comprises:
extracting a plurality of bamboo fibres from natural bamboo by means of mechanical extraction; and
impregnating said plurality of bamboo fibres with a binding matrix.

14. A paved surface (701) comprising a reinforcing structure (200, 300, 400, 500, 600, 703, 900, 1000) in accordance with claim 1; wherein
said reinforcing structure is positioned onto a first layer (702) of said paved surface and a second layer (704) is laid over said reinforcing structure.

## Patentansprüche

1. Eine Tragschichtbewehrung (200, 300, 400, 500, 600, 703, 900, 1000), die Folgendes beinhaltet:
eine erste Gruppe von Bündeln (201, 301, 402, 901, 1001), in der jedes besagtes Bündel im Wesentlichen parallel zu anderen Bündeln besagter erster Gruppe angeordnet ist;
eine zweite Gruppe von Bündeln (202, 302, 403, 902, 1002), die im Wesentlichen senkrecht zu besagter erster Gruppe von Bündeln angeordnet ist;
besagte erste Gruppe von Bündeln und besagte zweite Gruppe von Bündeln sind in einem Raster (203, 303, 401, 501, 601) angeordnet, das Öffnungen (204, 304, 1003) mit einer jeweiligen Breite (203, 305) und Länge (206, 306) von über 0,004 Metern umgrenzt; und wobei
besagte Tragschichtbewehrung des Weiteren eine Verbindungsvorrichtung (207, 307, 407, 903) beinhaltet, die besagte erste Gruppe von Bündeln und besagte zweite Gruppe von Bündeln in besagtem Raster hält; **dadurch gekennzeichnet, dass**
jedes besagte Bündel eine Vielzahl von Strängen (212, 905) aus aus Bambus gewonnenem Material beinhaltet und jedes besagte Bündel zum physikalischen und chemischen Schutz besagter Stränge mit einer Beschichtung (211, 906) versehen ist.

2. Eine Tragschichtbewehrung gemäß Patentanspruch 1, wobei besagte Tragschichtbewehrung als Materialrolle geformt ist.

3. Eine Tragschichtbewehrung gemäß Patentanspruch 1, wobei besagte Bündel besagte Stränge aus aus Bambus gewonnenem Material beinhalten und des Weiteren aus einem zweiten Material geformte Stränge beinhalten.

4. Eine Tragschichtbewehrung gemäß Patentanspruch 3, wobei besagtes zweites Material aus mindestens einem Mitglied der aus folgenden Stoffen bestehenden Gruppierung ausgewählt wird: Glasfasern, Viskosefasern und Kohlenstofffasern.

5. Eine Tragschichtbewehrung gemäß Patentanspruch 1, die des Weiteren eine erste an eine erste Seite (503) besagten Rasters angebrachte Tragschicht (404, 502) beinhaltet.

6. Eine Tragschichtbewehrung gemäß Patentanspruch 1, wobei besagte Beschichtung (211) aus mindestens einem Mitglied der aus folgenden Stoffen bestehenden Gruppierung ausgewählt wird: ein polymerer Werkstoff, ein elastomerer Werkstoff, natürlich vorkommendes Polymer, polymermodifizierter Asphalt, Synthetikkautschuk, natürlich vorkommender Bambussaft, natürlich vorkommendes Bambusharz, eine Naturkautschukkomponente, Epoxidharz und pflanzlich gewonnenes Epoxidharz.

7. Eine Tragschichtbewehrung gemäß Patentanspruch 1, wobei besagte Stränge eine erste Vielzahl von Bambusfasern (905) beinhalten und besagte Beschichtung eine Bindematrix (906) beinhaltet.

8. Eine Tragschichtbewehrung gemäß Patentanspruch 7, wobei besagte erste Vielzahl von Bambusfasern eine zweite Vielzahl von Bambusfasern beinhaltet und in der jede der besagten Vielzahl von Bambusfasern an eine andere aus besagter zweiter Vielzahl von Bambusfasern mittels besagter Bindematrix gebunden ist.

9. Eine Tragschichtbewehrung gemäß Patentanspruch 7, wobei besagte Verbindungsvorrichtung besagte Bindematrix (906) beinhaltet.

10. Eine asphaltierte Oberfläche (701), die eine Tragschichtbewehrung (200, 300, 400, 500, 600, 703, 900, 1000) gemäß einem jeden der vorstehenden Patentansprüche beinhaltet.

11. Ein Verfahren für die Fertigung einer Tragschichtbewehrung (200, 300, 400, 500, 600, 703, 900, 1000), das folgende Ablaufschritte beinhaltet:
Beschaffung einer Vielzahl von Strängen (212, 905) aus aus Bambus gewonnenem Material;
Verbindung einer Vielzahl von Strängen miteinander, um eine erste Gruppe von Bündeln (201, 301, 402, 901, 1001) und eine zweite Gruppe von Bündeln (202, 302, 403, 902, 1002) zu bilden;
derartige Anordnung besagter erster Gruppe von Bündeln, dass jedes besagte Bündel im Wesentlichen parallel zu einem entsprechenden Bündel ist;
Anordnung besagter zweiter Gruppe im Wesentlichen senkrecht zu besagter erster Gruppe von Bündeln;
Anordnung besagter erster Gruppe von Bündeln und besagter zweiter Gruppe von Bündeln in einem Raster (203, 303, 401, 501, 601), das Öffnungen (204, 304, 1003) mit einer jeweiligen Breite (205, 305) und Länge (206, 306) von über 0,004 Metern umgrenzt;
Verbindung besagter erster Gruppe von Bündeln und besagter zweiter Gruppe von Bündeln miteinander, damit besagtes Raster erhalten bleibt; und
Aufbringen einer Beschichtung (211, 906) auf besagten Bündeln zum physikalischen und chemischen Schutz besagter Stränge.

12. Ein Verfahren zur Fertigung einer Tragschichtbewehrung gemäß Patentanspruch 11, wobei besagte Vielzahl von Strängen eine Vielzahl von Bambusfasern beinhaltet und besagter Schritt der Verbindung besagter Vielzahl von Strängen miteinander Folgendes beinhaltet:
derartige Verfeinerung besagter Vielzahl von Bambusfasern, dass die Fasern in besagter Vielzahl von Bambusfasern im Wesentlichen aneinandergereiht sind.

13. Ein Verfahren zur Fertigung einer Tragschichtbewehrung gemäß Patentanspruch 12, wobei besagter Schritte des Aufbringens einer Beschichtung auf besagten Bündeln Folgendes beinhaltet:
Gewinnung einer Vielzahl von Bambusfasern aus natürlichem Bambus mittels mechanischer Extraktion; und
Imprägnierung besagter Vielzahl von Bambusfasern mit einer Bindematrix.

14. Eine befestigte Oberfläche (701), die eine Tragschichtbewehrung (200, 300, 400, 500, 600, 703, 900, 1000) gemäß Patentanspruch 1 beinhaltet; wobei
besagte Tragschichtbewehrung auf einer ersten Schicht (702) besagter befestigter Oberfläche platziert wird und eine zweite Schicht (704) über besagte Tragschichtbewehrung gelegt wird.

## Revendications

1. Une structure de renforcement (200, 300, 400, 500, 600, 703, 900, 1000), comprenant :
un premier jeu de faisceaux (201, 301, 402, 901, 1001), chacun desdits faisceaux étant disposé de façon substantiellement parallèle à d'autres faisceaux dudit premier jeu ;
un deuxième jeu de faisceaux (202, 302, 403, 902, 1002) disposé de façon substantiellement perpendiculaire audit premier jeu de faisceaux ;
lesdits premier et deuxième jeux de faisceaux étant disposés sous forme de réseau (203, 303, 401, 501, 601) définissant des trous (204, 304, 1003) dont les largeurs (205, 305) et les longueurs (206, 306) sont supérieures à 0,004 mètre ; et
ladite structure de renforcement comprenant en outre un dispositif de raccordement (207, 307, 407, 903) maintenant lesdits premier et deuxième jeux de faisceaux dans ledit réseau ; **caractérisée par le fait que**
chacun desdits faisceaux comprend une série de brins (212, 905) d'une matière dérivée du bambou, chacun étant recouvert d'un revêtement (211, 906) assurant la protection physique et chimique desdits brins.

2. Une structure de renforcement selon la revendication 1, ladite structure de renforcement étant formée sous forme d'un rouleau de matière.

3. Une structure de renforcement selon la revendication 1, lesdits faisceaux comprenant lesdits brins de matière dérivée du bambou, ainsi que des brins formés avec une deuxième matière.

4. Une structure de renforcement selon la revendication 3, ladite deuxième matière étant sélectionnée parmi au moins un membre du groupe composé de fibres de verre, de fibres de viscose et de fibres de carbone.

5. Une structure de renforcement selon la revendication 1, comprenant en outre une première couche porteuse (404, 502) fixée sur un premier côté (503) dudit réseau.

6. Une structure de renforcement selon la revendication 1, ledit revêtement (211) étant sélectionné parmi au moins un membre du groupe composé d'un matériau polymère, d'un matériau élastomère, d'un polymère présent naturellement, d'un bitume modifié par des polymères, d'un caoutchouc synthétique, de sève de bambou présente naturellement, de résine de bambou présente naturellement, d'un composant du caoutchouc naturel, de résines époxydes, et d'une résine époxyde végétale.

7. Une structure de renforcement selon la revendication 1, dans laquelle lesdits brins comprennent une première série de fibres de bambou (905) et ledit revêtement comprend une matrice liante (906).

8. Une structure de renforcement selon la revendication 7, dans laquelle ladite première série de fibres de bambou comprend une deuxième série de fibres de bambou, et dans laquelle chacune de la deuxième série desdites fibres de bambou est liée à une autre de ladite deuxième série de fibres de bambou par ladite matrice liante.

9. Une structure de renforcement selon la revendication 7, dans laquelle ledit dispositif de raccordement comprend ladite matrice liante (906).

10. Une surface de revêtement bitumineux (701) comprenant une structure de renforcement (200, 300, 400, 500, 600, 703, 900, 1000) selon une quelconque des revendications précédentes.

11. Une méthode de fabrication d'une structure de renforcement (200, 300, 400, 500, 600, 703, 900, 1000), comprenant les étapes suivantes :
réalisation d'une série de brins (212, 905) d'une matière dérivée du bambou ;
combinaison d'une série de brins pour la formation d'un premier jeu de faisceaux (201, 301, 402, 901, 1001) et d'un deuxième jeu de faisceaux (202, 302, 403, 902, 1002) ;
aménagement dudit premier jeu de faisceaux de sorte que chaque faisceau soit substantiellement parallèle à un faisceau correspondant ;
aménagement dudit deuxième jeu de faisceaux de sorte que chaque faisceau soit substantiellement perpendiculaire audit premier jeu de faisceaux ;
aménagement desdits premier et deuxième jeux de faisceaux forme de réseau (203, 303, 401, 501, 601) définissant des orifices (204, 304, 1003) dont les largeurs (205, 305) et les longueurs (206, 306) sont supérieures à 0,004 mètre ;
raccordement desdits premier et deuxième jeux de faisceaux afin de maintenir ledit réseau ; et
application sur lesdits faisceaux d'un revêtement (211, 906) assurant la protection physique et chimique desdits brins.

12. Une méthode de fabrication d'une structure de renforcement selon la revendication 11, dans laquelle ladite série de brins comprend une série de fibres de bambou, et ladite étape de combinaison de ladite série de brins comprend :
le raffinage de ladite série de brins de sorte que les fibres de ladite série de fibres de bambou soient substantiellement alignées.

13. Une méthode de fabrication d'une structure de renforcement selon la revendication 12, dans laquelle ladite étape d'application d'un revêtement sur lesdits faisceaux comporte :
l'extraction d'une série de fibres de bambou de bambou naturel par extraction mécanique ; et
l'imprégnation de ladite série de fibres de bambou avec une matrice liante.

14. Une surface asphaltée (701) comprenant une structure de renforcement (200, 300, 400, 500, 600, 703, 900, 1000) selon la revendication 1 ; dans laquelle
ladite structure de renforcement est positionnée sur une première couche (702) de ladite surface asphaltée et une deuxième couche (704) est posée sur ladite structure de renforcement.
